

1

3,759,758  
**HIGH STRENGTH ALUMINUM CASTING ALLOY**  
Ikuo Hatano, Kyuya Oida, Tatuo Abe, Seiji Kumagai,  
Sueo Ojima, and Hiroshi Nagaeda, Aichi, Japan, as  
signors to Sumitomo Chemical Co., Ltd., Osaka, Japan  
No Drawing. Filed May 13, 1970, Ser. No. 37,000  
Claims priority, application Japan, May 13, 1969,

44/37,157

Int. Cl. C22f 1/04

U.S. CL. 148—159

4 Claims

## ABSTRACT OF THE DISCLOSURE

An aluminum casting alloy having good mechanical properties is prepared by adding, to aluminum, copper, 15 magnesium, and cadmium and, additionally, if desired, titanium and boron, and, additionally, if desired, manganese and silver, solution-heat-treating thereof at a temperature higher than 500° C., and then ageing the solution-heat-treated alloy at a temperature between 160° C. 20 and 190° C. for 4 to 48 hours. The alloy is useful in various types of machine members, aircraft, rolling-stock members, architectural members, and other structural appliances.

## BACKGROUND OF THE INVENTION

### Field of the invention

This invention relates to a high strength aluminum alloy, and more particularly to aluminum alloys having a high tensile strength, a high yield strength and excellent toughness and also to methods for producing them.

### Description of the prior art

Recently, aluminum alloys having excellent mechanical properties have been needed by the various industrial fields, such as the automobile, aircraft and building industries.

Relatively high strength can be obtained by wrought aluminum alloys, but satisfactory strength can hardly be obtained by casting aluminum alloys.

A few aluminum casting alloys have a tensile strength of about 40 kg./mm.<sup>2</sup> have already been well known, but alloys having a tensile strength of 45 kg./mm.<sup>2</sup> or more are only the aluminum-zinc-magnesium system alloy.

Alloys containing a relatively high amount of zinc are very susceptible to stress corrosion cracking. An aluminum-copper-magnesium-silver casting alloy disclosed in British Pat. No. 1,090,960 has a high tensile strength of 45 kg./mm.<sup>2</sup> or more, but this alloy is very expensive due to its containing silver. Therefore, the development of inexpensive aluminum casting alloys having a high tensile strength of 45 kg./mm.<sup>2</sup> or more, and favorable other mechanical properties, have long been desired.

As the result of extensive studies on aluminum casting alloys having high tensile strengths, high yield strengths and toughness, and desirable resistance to hot tearing and stress corrosion cracking, it was found that aluminum-copper-magnesium-cadmium casting alloys had the aforementioned requirements.

## SUMMARY OF THE INVENTION

It has been known that conventional aluminum-copper-magnesium alloys have obtained relatively high mechanical properties by heat treatment. The mechanical properties of these alloys can be remarkably improved by the addition of small amounts of cadmium and by suitable heat treatment; that is to say, to obtain alloys having a tensile strength, a yield strength and elongation of at least 45 kg./mm.<sup>2</sup>, at least 40 kg./mm.<sup>2</sup> and from 4 to 10%, respectively. These mechanical properties are comparable

2

with those of the expensive aluminum-copper-magnesium-silver alloys.

The age hardenable alloy of the present invention comprises 4.0 to 6.2% copper, 0.2 to 0.5% magnesium, 0.05 to 0.8% cadmium, 0.01 to 0.5% titanium and 0.001 to 0.01% boron, the remainder being aluminum.

The aluminum alloy of the present invention is solution-heat-treated at a temperature greater than 500° C. and aged at a temperature of from 160 to 190° C. for from 4 to 48 hours.

## DETAILED DESCRIPTION OF THE PREFERRED EMBODIMENTS

The amount of the alloying elements added to the aluminum casting alloy is within the aforesaid ranges for the following reasons.

Copper addition is essential in order to increase the strength of the alloy. Copper in an amount of from 4.0 to 6.2% is required for this purpose. The addition of copper in an amount of more than 6.2% increases the phase which is insoluble in the matrix even by the solution heat treatment, and therefore is unfavorable in order to keep the good mechanical properties and to decrease the tendency of the alloy to undergo hot tearing. For optimum results, the copper is present in an amount of from 4.7 to 5.5%.

The addition of magnesium increases the strength and the ageing property of the alloy. Magnesium in an amount of from 0.2 to 0.5% is required for this purpose. The addition of magnesium in an amount of more than 0.5% increases the tendency of the alloy to undergo hot tearing and often causes burning and quench cracking if the solution heat treatment temperature is higher, while the strength decreases if the lower solution heat treatment temperature is utilized to prevent the occurrence of hot tearing. For optimum results, the magnesium is present in an amount of from 0.2 to 0.4%.

The addition of a small amount of cadmium in the aluminum-copper-magnesium alloy remarkably increases the age hardening property and the mechanical properties of the alloy, and also improves the resistance of the alloy to stress corrosion cracking. Cadmium in an amount of from 0.05 to 0.8% is required for this purpose. The addition of cadmium in an amount of more than 0.8% increases the hot tearing tendency burning during the solution heat treatment and quenching cracking. For optimum results, the cadmium is present in an amount of from 0.1 to 0.2%. It is noteworthy that cadmium is far cheaper than silver and therefore this aluminum-copper-magnesium-cadmium alloy can be produced at far lower cost than alloys containing silver.

Titanium is beneficial in assuring both fine grain structure in the alloy and good mechanical properties through successful heat solution treatment, and in order to prevent the cause of hot tearing. Titanium in an amount of 0.01 to 0.5% is required for this purpose. The addition of titanium in an amount of more than 0.5% causes the precipitation of gross compounds which reduce the mechanical properties. For optimum results, the titanium is present in an amount of from 0.1 to 0.3%.

Boron, in an amount of from 0.001 to 0.01%, added to the alloy together with the titanium through the mother alloy or the flux, is beneficial in assuring fine grain structure.

The properties of the alloy are further improved by the addition of silver and manganese to the aluminum-copper-magnesium-cadmium alloy. The addition of a small amount of silver further increases the age-hardening properties and the mechanical properties of the alloy. That is to say, an alloy having a tensile strength of 50

kg./mm.<sup>2</sup> or more, a yield strength of 45 kg./mm.<sup>2</sup> or more and an elongation of 4 to 15% can be obtained. The addition of silver in an amount below 2.0% improves the mechanical properties. However, the addition of silver in an amount more than 2.0% has no more effect on the improvement of the mechanical properties. Since silver is an expensive metal, it is preferable that the amount of silver in the alloy be below 2.0%. Although the cost of the alloy becomes higher by the addition of silver, a casting requiring especially high strength can overcome such a difficult requirement.

The addition of manganese improves the resistance of the alloy to stress corrosion cracking. That is to say, the addition of manganese in an amount of below 1% increases the resistance to stress corrosion cracking without decreasing the mechanical properties, but an amount of manganese greater than 1% does not have the desired effect. For optimum results, the manganese is present in an amount of below 0.5%.

It is desirable to use aluminum of as high a purity as possible for the production of the aluminum-copper-magnesium-cadmium alloy in order to obtain an alloy having high strength and toughness; the iron and silicon content of the alloy are desirable below 0.2%. The optimum ranges of the content of the alloying elements of the alloy are as follows:

|           | Percent    |
|-----------|------------|
| Copper    | 4.7 to 5.5 |
| Magnesium | 0.2 to 0.4 |
| Cadmium   | 0.1 to 0.2 |
| Titanium  | 0.1 to 0.3 |
| Boron     | Below 0.01 |

The aluminum alloy of the present invention is heat-treated in the following manner.

The solution heat treatment must be carried out at a temperature higher than 500° C. and for a time sufficient to dissolve the deposited copper-rich compound fully and uniformly into the matrix. The solution heat-treating temperature is preferably selected as high as possible without causing burning or quench cracking. The upper limit of the solution heat-treating temperature is determined by the content of the alloying elements, especially cadmium and magnesium. The aluminum alloy having the above preferred composition is satisfactorily solution-heat-treated at 530° C. for 12 hours.

The water quenching after the solution heat treatment must be carried out as rapidly as possible. The temperature of the water after quenching must not exceed 50° C. The quenching temperature for intricate castings having parts of different thicknesses is preferably 5° to 10° C. lower than the ordinary solution heat-treating temperature, thus preventing internal strain or cracking during the quenching operation.

The precipitation heat treatment of this aluminum alloy is carried out at a temperature of about 160° to 190° C. for 4 to 48 hours.

Maximum strength is obtained by ageing at 175° C. for 20 hours. A high yield strength is obtained by ageing for a longer time at a higher temperature, whereas a high elongation is obtained by ageing for a shorter time at a lower temperature.

In the case of requiring a high elongation while sacrific-

ing the yield strength, the ageing temperature must not exceed 160° C.

The following examples illustrate the present invention but should not be construed as limiting the scope of the invention in any way.

#### EXAMPLE 1

Aluminum of 99.9% purity was cleaned to remove the machine oil and smut, dried and was charged into a graphite crucible and melted therein. After the temperature of the melt had reached 750° C., an aluminum-5% titanium mother alloy was added to the melt. Then, copper was added to the melt at 750° C. and the melt was stirred. After that, cadmium wrapped in aluminum foil and magnesium were added to the melt at 730° C. and 750° C., respectively.

A flux containing titanium and boron  
(K<sub>2</sub>TiF<sub>6</sub>+KBF<sub>4</sub>+C<sub>2</sub>Cl<sub>6</sub>)

20 was further added to the melt at 750° C. in amounts of 0.1 to 0.2% based on the weight of the melt for refining the grain structure of the alloy. Finally, hexachloroethane pills (C<sub>2</sub>Cl<sub>6</sub>) were plunged into the melt by means of a phosphorizer to degass the melt.

25 The resultant melt held at 750° C. for 30 minutes was subjected to a gas generating test by pouring about 200 g. of the melt into a preheated isolite mold, solidifying the melt under a reduced pressure of about 5 mm. Hg, and observing the generation of gas from the solidifying melt.

30 After confirming the lack of gas generation by means of the test, the dross was removed from the melt surface and the melt was poured into a test permanent mold. The casting test pieces were solution-heat-treated at 530° C. for 12 hours, quenched into cold water and aged at 165° C. for 32 hours.

35 The test pieces were subjected to a tensile test and chemical analysis.

40 The results were as follows; tensile strength 48.6 kg./mm.<sup>2</sup> yield strength (0.2% offset) 43.6 kg./mm.<sup>2</sup>; elongation 6.0%; chemical composition; Cu 5.37%, Mg 0.33%, Cd 0.13%, Ti 0.16%, B 0.004%, Fe 0.07%, Si 0.05%, and balance Al.

#### EXAMPLE 2

45 An aluminum alloy melt was produced according to the same melting and alloying procedures as in Example 1. Gas was removed from the melt by injecting a gas mixture of chlorine and nitrogen through the melt with a graphite pipe. The test pieces cast in the mold were solution-heat-treated at 525° C. for 6 hours, quenched into cold water and aged at 180° C. for 16 hours. The tensile strength, yield strength (0.2% offset), elongation and chemical composition of the resultant alloy were as follows: tensile strength 47.0 kg./mm.<sup>2</sup>; yield strength 40.6 kg./mm.<sup>2</sup>; elongation 9.6%; chemical composition; Cu 4.83%, Mg 0.31%, Cd 0.11%, Ti 0.02%, B 0.003%, Fe 0.07%, Si 0.04% and balance Al.

50 The titanium in the alloy was derived not from the aluminum-titanium alloy but from the refining flux.

55 Table 1 shows the chemical compositions of aluminum alloys of this invention and those of conventional high strength and heat resistant aluminum casting alloys.

TABLE 1.—CHEMICAL COMPOSITION

| Alloy No.       | Cu   | Mg   | Cd    | Ti   | B     | Fe    | Si    | Ni    | Mn    | Ag    | Al       |
|-----------------|------|------|-------|------|-------|-------|-------|-------|-------|-------|----------|
| 3               | 4.99 | 0.30 | 0.17  | 0.16 | 0.003 | 0.07  | 0.04  | ..... | ..... | ..... | Balance. |
| 4               | 5.77 | 0.34 | 0.14  | 0.16 | 0.004 | 0.07  | 0.05  | ..... | ..... | ..... | Do.      |
| 5               | 4.25 | 0.40 | 0.28  | 0.18 | 0.002 | 0.08  | 0.04  | ..... | ..... | ..... | Do.      |
| 6               | 4.15 | 0.30 | 0.59  | 0.16 | 0.003 | 0.07  | 0.05  | ..... | ..... | ..... | Do.      |
| 7               | 4.66 | 0.29 | 0.14  | 0.32 | 0.003 | 0.09  | 0.05  | ..... | ..... | ..... | Do.      |
| 8               | 5.11 | 0.30 | 0.10  | 0.21 | 0.004 | 0.07  | 0.04  | ..... | 0.60  | ..... | Do.      |
| 9               | 4.97 | 0.34 | 0.10  | 0.17 | 0.003 | 0.07  | 0.04  | 0.31  | ..... | ..... | Do.      |
| 10              | 5.16 | 0.31 | 0.16  | 0.17 | 0.003 | 0.07  | 0.04  | 0.32  | 0.60  | ..... | Do.      |
| 11 <sup>1</sup> | 4.34 | 0.31 | ..... | 0.16 | ..... | 0.17  | 0.20  | ..... | ..... | ..... | Do.      |
| 12 <sup>1</sup> | 4.68 | 0.37 | ..... | 0.14 | ..... | 0.06  | 0.04  | ..... | ..... | ..... | Do.      |
| 13 <sup>1</sup> | 5.02 | 0.30 | ..... | 0.21 | 0.002 | 0.06  | 0.03  | ..... | 0.61  | ..... | Do.      |
| 14 <sup>1</sup> | 5.00 | 0.28 | ..... | 0.19 | 0.003 | 0.002 | 0.002 | 0.60  | ..... | ..... | Do.      |
| 15 <sup>1</sup> | 1.03 | 1.08 | ..... | 0.07 | ..... | 0.32  | 11.97 | 1.64  | 0.01  | ..... | Do.      |

<sup>1</sup> Conventional aluminum alloys.

Table 2 shows the heat treatment conditions and the mechanical properties at room temperature of the alloys tabulated in Table 1.

TABLE 2.—HEAT TREATMENT CONDITIONS AND MECHANICAL PROPERTIES AT ROOM TEMPERATURE

| Alloy No.       | Solution heat treatment | Quenching liquid | Ageing treatment  | Tensile strength, kg./mm. <sup>2</sup> | Yield strength, kg./mm. <sup>2</sup> | Elongation, percent |
|-----------------|-------------------------|------------------|-------------------|----------------------------------------|--------------------------------------|---------------------|
| 3               | 530° C. X8 hours        | Cold water       | 165° C. X28 hours | 47.6                                   | 41.7                                 | 8.7                 |
| 4               | 530° C. X12 hours       | do               | 165° C. X32 hours | 47.5                                   | 42.3                                 | 5.0                 |
| 5               | 520° C. X6 hours        | do               | 175° C. X20 hours | 46.0                                   | 40.6                                 | 7.2                 |
| 6               | do                      | do               | 180° C. X16 hours | 45.1                                   | 39.1                                 | 8.1                 |
| 7               | 530° C. X12 hours       | do               | 165° C. X28 hours | 45.9                                   | 39.7                                 | 10.2                |
| 8               | do                      | do               | 165° C. X24 hours | 51.8                                   | 46.9                                 | 9.5                 |
| 9               | do                      | do               | 165° C. X28 hours | 46.8                                   | 39.7                                 | 7.8                 |
| 10              | do                      | do               | 165° C. X24 hours | 51.0                                   | 46.2                                 | 8.6                 |
| 11 <sup>1</sup> | 515° C. X6 hours        | do               | 170° C. X12 hours | 40.4                                   | 33.3                                 | 8.2                 |
| 12 <sup>1</sup> | 530° C. X4 hours        | do               | 175° C. X16 hours | 42.1                                   | 34.4                                 | 11.1                |
| 13 <sup>1</sup> | 525° C. X12 hours       | do               | 160° C. X20 hours | 47.0                                   | 41.5                                 | 10.4                |
| 14 <sup>1</sup> | do                      | do               | do                | 48.3                                   | 43.9                                 | 7.2                 |
| 15 <sup>1</sup> | 520° C. X6 hours        | 70° C. Xwater    | 170° C. X15 hours | 35.9                                   | 35.9                                 | 0.4                 |

<sup>1</sup> Conventional aluminum alloys.

Table 3 shows the mechanical properties at elevated temperature of the alloys shown in Tables 1 and 2.

TABLE 3.—MECHANICAL PROPERTIES AT Elevated TEMPERATURE

| Alloy No. | Mechanical properties      |         |         |         |      |
|-----------|----------------------------|---------|---------|---------|------|
|           | 100° C.                    | 200° C. | 250° C. | 300° C. |      |
| 3         | T.S., kg./mm. <sup>2</sup> | 43.4    | 34.6    | 26.6    | 18.6 |
|           | Y.S., kg./mm. <sup>2</sup> | 40.8    | 34.5    | 26.5    | 17.6 |
|           | E., percent                | 9.8     | 9.7     | 9.3     | 9.1  |
| 13 *      | T.S., kg./mm. <sup>2</sup> | 42.0    | 34.4    | 26.9    | 18.4 |
|           | Y.S., kg./mm. <sup>2</sup> | 38.6    | 33.7    | 26.5    | 17.8 |
|           | E., percent                | 10.9    | 10.7    | 10.1    | 10.6 |
| 15 *      | T.S., kg./mm. <sup>2</sup> | 32.5    | 31.0    | 25.8    | 16.5 |
|           | Y.S., kg./mm. <sup>2</sup> | 32.5    | 29.8    | 24.4    | 15.2 |
|           | E., percent                | 0.4     | 0.7     | 1.3     | 3.2  |

It is evident from Tables 2 and 3 that the aluminum alloy of the present invention has excellent mechanical properties not only at room temperature but also at elevated temperatures.

As mentioned above, the aluminum casting alloy of this invention can be produced at low cost and has excellent mechanical properties as compared with those of conventional aluminum alloys, and therefore can be applied to various types of uses; e.g., as machine members, aircraft members, rolling-stock members, architectural members and other structural appliances.

What is claimed is:

1. A high strength aluminum casting alloy consisting of from 4.7 to 5.5% copper, from 0.2 to 0.4% magnesium, from 0.1 to 0.2% cadmium, from 0.1 to 0.3% titanium and not more than 0.01% boron, not more than 0.5% manganese, not more than 0.2% iron and silicon, the balance being aluminum,

said alloy having been solution-heat treated at a temperature of at least 500° C., and for a time sufficient to dissolve the deposited copper-rich compounds into the matrix of said alloy, and subsequently aged at a temperature of from 160° C. to 190° C., for a period of time ranging from 4 to 48 hours.

2. A method of heat-treating a high strength aluminum casting alloy, said alloy consisting of from 4.7 to 5.5% copper, from 0.2 to 0.4% magnesium, from 0.1 to 0.2%

cadmium, and not more than 0.1% boron, not more than 0.5% manganese, the balance being aluminum, said method comprising solution-heat treating said alloy at a temperature of at least 500° C. and for a time sufficient to dissolve the deposited copper-rich compounds into the matrix of said alloy, quenching said alloy and then ageing said alloy at a temperature of from 160 to 190° C., and for a period of time of from 4 to 48 hours.

3. A method of heat-treating a high strength aluminum casting alloy, said alloy consisting of from 4.7 to 5.5% copper, from 0.2 to 0.4% magnesium, from 0.1 to 0.2% cadmium, from 0.1 to 0.3% titanium, not more than 0.01% boron, not more than 0.5% manganese, not more than 0.2% iron and silicon, the balance being aluminum,

said method comprising solution-heat-treating said alloy at a temperature of at least 500° C. and for a period of time sufficient to dissolve the deposited copper-rich compounds into the matrix of said alloy, quenching said alloy in cold water wherein the temperature of the water after quenching does not exceed 50° C., and ageing said alloy at a temperature between 160 and 190° C. for from 4 to 48 hours.

4. The method as in claim 3, wherein the temperature of said solution-heat-treatment varies from 520 to 530° C. for a period of time of between 6 and 12 hours, and wherein said ageing varies from a temperature of 165 to 180° C. for a period of time of 16 to 32 hours.

#### References Cited

#### UNITED STATES PATENTS

- |           |         |               |        |
|-----------|---------|---------------|--------|
| 3,287,185 | 11/1966 | Vachet et al. | 75—142 |
| 3,347,665 | 10/1967 | Miller et al. | 75—142 |
| 3,414,406 | 12/1968 | Doyle et al.  | 75—142 |
| 3,475,166 | 10/1969 | Raffin        | 75—142 |

RICHARD O. DEAN, Primary Examiner

U.S. CL. X.R.

75—142; 148—32.5